# EUROPEAN PATENT SPECIFICATION

(11) **EP 1 904 713 B1**
(45) Date of publication and mention of the grant of the patent: **09.09.2009**
(21) Application number: 06787231.7
(22) Date of filing: 14.07.2006
(51) Int. Cl.: E21B 10/08, E21B 10/20, E21B 10/22

(54) **SYSTEM5 METHOD, AND APPARATUS FOR REDUCING RESIDUAL STRESS IN AS-WELDED ROLLER CONE BIT BALL PLUG WELDS**
SYSTEM, VERFAHREN UND VORRICHTUNG ZUR REDUZIERUNG VON RESTSPANNUNGEN IN ROLLENBOHRMEISSELKUGELSTOPFENSCHWEISSUNGEN IM GESCHWEISSTEN ZUSTAND
PROCEDE, SYSTEME ET APPAREIL PERMETTANT DE REDUIRE LES CONTRAINTES RESIDUELLES DANS LES SOUDURES D'UN ARRET DE BILLE DE TREPAN A MOLETTES CONIQUES SOUDE

(30) Priority: 15.07.2005 US 183121
(43) Date of publication of application: 02.04.2008
(62) Divisional of application: 09007819.7
(73) Proprietor: Baker Hughes Incorporated, Houston, TX 77019 (US)
(72) Inventor: ZAHRADNIK, Anton, F., Sugar Land, TX 77479 (US); JONES, Ronnie, L., New Waverly, TX 77358 (US); NGUYEN, Don Q., Houston, Texas 77066 (US); RICKS, Gregory L., Spring, Texas 77386 (US); BEUERSHAUSEN, Christopher C., Magnolia, Texas 77354 (US); Sullivan, Eric C., Houston, Texas 77089 (US)
(74) Representative: Jeffrey, Philip Michael
(86) International application number: PCT/US2006/027294
(87) International publication number: WO 2007/011686

(56) References cited:
- WO-A-99/39075
- JP-A- 11 209 825
- US-A- 3 158 214
- US-A- 3 989 315
- US-A1- 2004 250 584

## Description

The present invention relates in general to stress reduction in roller cone bits and, in particular, to an improved system, method, and apparatus for reducing residual stress in as-welded roller cone bit ball plug welds.

Rotary-type drill bits include both rotary drag bits and roller- cone bits. In a roller-cone arrangement, the bit typically has three cones, each independently rotatable with respect to the bit body supporting the cones through bearing assembles. The cones carry either integrally formed teeth or separately formed inserts that provide the cutting action of the bit.

Roller cone bits typically use a ball retention system for securing the cones to the heads. The retention system includes a radial ball race incorporated into each cone and the head bearings. A ball way is provided between the head ball race and the head outer diameter (OD) to facilitate assembly. When the cone is mated to the head, the respective ball races are aligned and, together, they define a toroidal space. Ball bearings are introduced via the ball way into the space. A ball plug is then inserted into the ball way to block the discontinuity (i.e., the hole) in the head ball race and to ensure that the ball bearings are retained in the race. The ball plug is secured to the head OD by welding, e.g. as described in WO 99/39075 where the bal plug weld is formed from multiple layers of material. US 3,989,315 discloses another method of retaining the ball plug in the ball way using an assembly comprising a hollow cup and a plug.

While cooling from welding, residual stress can accumulate in the weld region (e.g., the fusion and heat-affected zones). Depending upon the orientation and magnitude of the residual stress, the service load capacity of the assembly can be significantly reduced. This structural configuration gives rise to one type of head section failure, which includes cracks that initiate at the root of the ball plug weld and then propagate toward the head OD, and then turn and propagate toward the base of the bearing pin. Solutions for addressing this problem would be desirable.

According to a first aspect of the present invention, there is provided a method of reducing residual stress in a roller cone bit as claimed in claim 1.

According to a second aspect of the present invention, there is provided a roller cone bit as claimed in claim 12.

In the present invention, material is selectively removed from the weld, and preferably from the heat-affected zone and/or the surrounding area, to promote relaxation of residual stress. In other embodiments, deflection is also imposed and/or heat or vibration is also applied to promote relaxation. By reducing weld area residual stress with the present invention, service load capacity and/or service life is increased.

The foregoing and other objects and advantages of the present invention will be apparent to those skilled in the art, in view of the following detailed description of the present invention, taken in conjunction with the appended claims and the accompanying drawings.

So that the manner in which the features and advantages of the invention, as well as others which will become apparent are attained and can be understood in more detail, more particular description of the invention briefly summarized above may be had by reference to the embodiment thereof which is illustrated in the appended drawings, which drawings form a part of this specification. It is to be noted, however, that the drawings illustrate only an embodiment of the invention and therefore are not to be considered limiting of its scope as the invention may admit to other equally effective embodiments.
Figure 1 is a half-sectional view of a first roller cone bit;
Figure 2 is an enlarged sectional view of a head and cone portion of the roller cone bit of Figure 1;
Figure 3 is an enlarged sectional view of a second roller cone bit; and
Figure 4 is a high level flow diagram of one embodiment of a method in accordance with the present invention.

Referring to Figures 1 and 2, a roller cone bit 11 is shown. Bit 11 comprises a bit body 13 having heads 15 (one shown) with cones 17. Each head 15 and cone 17 includes a retention system having a ball race 19 at an intersection between the head 15 and cone 17. A ball way 21 extends from the ball race 19 to an outer diameter (left sides of Figures 1 and 2) of the head 15. The outer diameter forms a portion of a perimeter area 23 of the head 15. The perimeter area 23 generally includes a region of the head 15 extending from the ball way 21 radially outward and axially inward with respect to the ball way 21.

The respective ball races 19a, 19b of the head 15 and cone 17 are aligned to define a toroidal space. Balls 25 are located in the ball race 19 for mechanically retaining the cone 17 on the head 15. A ball plug 27 is located in the ball way 21 to retain the balls 25 in the ball race 19. A barrier 29, in this case a weld, is formed adjacent the outer diameter of the head 15 to secure the ball plug 27 in the ball way 21.

The present invention also comprises stress reduction means for reducing residual stress at the barrier (weld) 29 and the perimeter area 23 of the head 15 adjacent the outer diameter to increase a service load capacity and a service life of the roller cone bit 11. The residual stress reduction is accomplished in the present invention, at least in part, by removing material from the barrier 29, such as by forming a hole 39 in the barrier 29 that extends in an axial direction with respect to the ball way 21. In other words, the stress reduction means comprises a void 39 (Figure 3) in the barrier 29. The void 39 may comprise a drilled hole that extends in an axial direction of the ball way 21.

In one embodiment, the stress reduction means further comprises an inner weld 31 (Figure 2) formed from a first material adjacent the ball plug 27. The weld 29 is formed on the inner weld 31 from a second material that has a higher strength than the first material. The first material may comprise many different materials, including nickel, nickel alloy, stainless steel, and inconel. The second material may comprise steel or the like.

In addition, a single weld having comprising one or more passes may be used as the barrier 29. These embodiments also may utilize a single material, such as nickel, to form the welds. Moreover, the entire weld may be formed from a single, softer material.

The residual stress reduction also may comprise a heat treatment that may be performed on the entire roller cone bit 11. As shown in Figure 3, the residual stress reduction may be localized and limited to the barrier 29 and the perimeter area 23, as with a small device 35 (e.g., a heat source, an ultrasonic tool, etc.) and a controller 37 for applying a heat treatment or an ultrasonic vibration treatment, respectively, to the barrier 29 and the perimeter area 23.

The present invention also comprises a method of reducing residual stress in a roller cone bit. As shown in Figure 4, one embodiment of the method starts as indicated at step 41, and comprises providing a roller cone bit with heads with cones (step 43); securing the cones to the heads with balls located in a ball race at an intersection between each cone and head, each ball race having a ball way extending from the ball race to a perimeter area of the head (step 45); installing a ball plug in each ball way to retain the balls in the ball race (step 47); forming a barrier at the perimeter area to retain the ball plug in the ball way (step 49); reducing residual stress at the barrier and the perimeter area to increase a service load capacity and a service life of the roller cone bit (step 51); before ending as indicated at step 53.

Step 51 comprises removing material from the barrier, such as by forming a hole in the barrier that extends in an axial direction of the ball way.

The method also may comprise forming an inner weld from a first material adjacent the ball plug, and forming an outer weld on the inner weld from a second material that has a higher strength than the first material. Step 51 may also comprise applying a heat treatment, such as by subjecting the ball plug to elevated temperatures during the stress relief operation. This embodiment may further comprise localizing the heat treatment to a limited portion of the roller cone bit including the barrier and the perimeter area, or subjecting the entire roller cone bit to the heat treatment. Step 51 also may comprise applying an ultrasonic vibration treatment the barrier and the perimeter area.

While the invention has been shown or described in only some of its forms, it should be apparent to those skilled in the art that it is not so limited, but is susceptible to various changes without departing from the scope of the invention as set forth in the accompanying claims.

## Claims

1. A method of reducing residual stress in a roller cone bit, the method comprising:
(a) providing a roller cone bit (11) with heads (15) with cones (17);
(b) securing the cones (17) to the heads (15) with balls (25) located in a ball race (19) at an intersection between each cone and head, each ball race (19) having a ball way (21) extending from the ball race to a perimeter area (23) of the head (15);
(c) installing a ball plug (27) in each ball way (21) to retain the balls (25) in the ball race (19); and
(d) forming a weld (29) at the perimeter area (23) to retain the ball plug (27) in the ball way (21); said method being **characterised by**:
(e) removing material from the weld (29).

2. A method according to claim 1, comprising forming an inner weld (31) from a first material adjacent the ball plug (27), and forming an outer weld (29) on the inner weld (31) from a second material that has a higher strength than the first material.

3. A method according to claim 2, wherein the first material is selected from the group consisting of: nickel; nickel alloy; stainless steel; and inconel, and the second material is steel

4. A method according to claim 1, wherein said weld (29) is formed with at least one pass from a single material.

5. A method according to any preceding claim, further comprising applying a heat treatment.

6. A method according to claim 5, further comprising subjecting the ball plug (27) to elevated temperatures during the heat treatment.

7. A method according to claim 5 or 6, further comprising localizing the heat treatment to a limited portion of the roller cone bit (11) including the weld (29) and the perimeter area (23).

8. A method according to claim 5, further comprising subjecting the entire roller cone bit (11) to the heat treatment.

9. A method according to any of claims 1 to 4, further comprising applying an ultrasonic vibration treatment to the barrier (29) and the perimeter area (23).

10. A method according to any preceding claim, wherein said step of removing material from the weld comprises forming a hole (39) in the weld (29) that extends in an axial direction of the ball way (21).

11. A method according to any preceding claim, wherein residual stress in the weld (29) and the perimeter area (23) is reduced to increase a service load capacity and a service life of the roller cone bit.

12. A roller cone bit, comprising:
a bit body (13) having heads (15) with cones (17), each head and cone including a ball race (19) at an intersection between the head (15) and cone (17), a ball way (21) extending from the ball race (19) to an outer diameter of the head (15), the respective ball races of the head and cone being aligned to define a toroidal space, balls (25) located in the ball race (19) for mechanically retaining the cone (15) on the head (17), a ball plug (27) located in the ball way (21) to retain the balls (25) in the ball race (19), and a weld (29) formed adjacent the outer diameter of the head (15) to secure the ball plug (27) in the ball way (21);
**characterised in that:**
said weld comprises a void (39).

13. A roller cone bit according to claim 12, wherein the void (39) in the weld (29) is a hole that extends in an axial direction of the ball way.

14. A roller cone bit according to claim 12 or 13, further comprising an inner weld (31) formed from a first material adjacent the ball plug (27), the weld (29) is formed on the inner weld (31) from a second material that has a higher strength than the first material.

15. A roller cone bit according to claim 14, wherein the first material is selected from the group consisting of: nickel; nickel alloy; stainless steel; and inconel, and the second material is steel.

## Patentansprüche

1. Verfahren zum Reduzieren von Restspannung in einem Rollenmeißel, wobei das Verfahren folgendes umfaßt:
(a) Bereitstellen eines Rollenmeißels (11) mit Köpfen (15) mit Kegeln (17);
(b) Sichern der Kegel (17) an den Köpfen (15) mit Kugeln (25) angeordnet in einem Kugelring (19) an einer Kreuzung zwischen jedem Kegel und Kopf, wobei jeder Kugelring (19) einen Kugelweg (21) aufweist, der sich von dem Kugelring zu einem Umfangsbereich (23) des Kopfs (15) erstreckt;
(c) Installieren eines Kugelstopfens (27) in jedem Kugelweg (21) zum Halten der Kugeln (25) in dem Kugelring (19) und
(d) Ausbilden einer Schweißstelle (29) am Umfangsbereich (23) zum Halten des Kugelstopfens (27) in dem Kugelweg (21); wobei das Verfahren **gekennzeichnet ist durch**:
(e) Entfernen von Material von der Schweißstelle (29).

2. Verfahren nach Anspruch 1, umfassend das Ausbilden einer inneren Schweißstelle (31) aus einem ersten Material bei dem Kugelstopfen (27) und Ausbilden einer äußeren Schweißstelle (29) an der inneren Schweißstelle (31) aus einem zweiten Material, das eine höhere Festigkeit als das erste Material aufweist.

3. Verfahren nach Anspruch 2, wobei das erste Material ausgewählt ist aus der Gruppe bestehend aus: Nickel; Nickellegierung; rostfreiem Stahl; und Inconel, und das zweite Material Stahl ist.

4. Verfahren nach Anspruch 1, wobei die Schweißstelle (29) mit mindestens einem Durchgang aus einem einzigen Material ausgebildet wird.

5. Verfahren nach einem vorhergehenden Anspruch, weiterhin umfassend das Anwenden einer Wärmebehandlung.

6. Verfahren nach Anspruch 5, weiterhin umfassend das Unterziehen des Kugelstopfens (27) erhöhten Temperaturen während der Wärmebehandlung.

7. Verfahren nach Anspruch 5 oder 6, weiterhin umfassend das Lokalisieren der Wärmebehandlung auf einen begrenzten Abschnitt des Rollenmeißels (11) einschließlich der Schweißstelle (29) und dem Umfangsbereich (23).

8. Verfahren nach Anspruch 5, weiterhin umfassend das Unterziehen des ganzen Rollenmeißels (11) der Wärmebehandlung.

9. Verfahren nach einem der Ansprüche 1 bis 4, weiterhin umfassend das Anwenden einer Ultraschallschwingungsbehandlung auf die Barriere (29) und den Umfangsbereich (23).

10. Verfahren nach einem vorhergehenden Anspruch,
wobei der Schritt des Entfernens von Material von der Schweißstelle das Ausbilden eines Lochs (39) in der Schweißstelle (29) umfaßt, das sich in einer axialen Richtung des Kugelwegs (21) erstreckt.

11. Verfahren nach einem der vorhergehenden Ansprüche,
wobei eine Restspannung in der Schweißstelle (29) und dem Umfangsbereich (23) reduziert wird, um die Nutzlastkapazität und die Nutzungsdauer des Rollenmeißels zu verlängern.

12. Rollenmeißel, umfassend:
einen Meißelkörper (13) mit Köpfen (15) mit Kegeln (17), wobei jeder Kopf und Kegel einen Kugelring (19) an einer Kreuzung zwischen dem Kopf (15) und
dem Kegel (17) enthält, wobei sich ein Kugelweg (21) von dem Kugelring (19) zu einem Außendurchmesser des Kopfs (15) erstreckt, wobei die jeweiligen Kugelringe des Kopfs und des Kegels ausgerichtet sind, um einen torusförmigen Raum zu definieren, wobei Kugeln (25) in dem Kugelring (19) angeordnet sind, um den Kegel (15) mechanisch an dem Kopf (17) festzuhalten, wobei ein Kugelstopfen (27) in dem Kugelweg (21) angeordnet ist, um die Kugeln (25) in dem Kugelring (19) festzuhalten, und eine Schweißstelle (29) bei dem Außendurchmesser des Kopfs (15) ausgebildet ist, um den Kugelstopfen (27) in dem Kugelweg (21) zu sichern;
**dadurch gekennzeichnet, daß:**
die Schweißstelle einen Hohlraum (39) umfaßt.

13. Rollenmeißel nach Anspruch 12, wobei der Hohlraum (39) in der Schweißstelle (29) ein Loch ist, das sich in einer axialen Richtung des Kugelwegs erstreckt.

14. Rollenmeißel nach Anspruch 12 oder 13, weiterhin umfassend eine aus einem ersten Material bei dem Kugelstopfen (27) ausgebildete innere Schweißstelle (31), wobei die Schweißstelle (29) an der inneren Schweißstelle (31) aus einem zweiten Material ausgebildet ist, das eine höhere Festigkeit als das erste Material aufweist.

15. Rollenmeißel nach Anspruch 14, wobei das erste Material ausgewählt ist aus der Gruppe bestehend aus: Nickel; Nickellegierung; rostfreiem Stahl; und Inconel, und das zweite Material Stahl ist.

## Revendications

1. Procédé permettant de réduire les contraintes résiduelles dans un trépan à molettes coniques, le procédé comprenant les étapes suivantes:
(a) fournir un trépan à molettes coniques (11) pourvu de têtes (15) comportant des cônes (17);
(b) fixer les cônes (17) aux têtes (15) avec des billes (25) situées dans une piste de roulement (19) à une intersection entre chaque cône et chaque tête, chaque piste de roulement (19) comprenant un chemin de bille (21) qui s'étend à partir de la piste de roulement jusqu'à une région périphérique (23) de la tête (15);
(c) installer un arrêt de bille (27) dans chaque chemin de bille (21) pour retenir les billes (25) dans la piste de roulement (19); et
(d) former une soudure (29) à la région périphérique (23) pour retenir l'arrêt de bille (27) dans le chemin de bille (21);
ledit procédé étant **caractérisé par**:
(e) enlever de la matière de la soudure (29).

2. Procédé selon la revendication 1, comprenant la formation d'une soudure intérieure (31) à partir d'une première matière à proximité de l'arrêt de bille (27), et la formation d'une soudure extérieure (29) sur la soudure intérieure (31) à partir d'une seconde matière dont la résistance est supérieure à celle de la première matière.

3. Procédé selon la revendication 2, dans lequel la première matière est sélectionnée dans le groupe comprenant le nickel, un alliage de nickel, l'acier inoxydable et l'inconel; et la seconde matière est l'acier.

4. Procédé selon la revendication 1, dans lequel ladite soudure (29) est formée avec au moins une passe à partir d'une seule matière.

5. Procédé selon l'une quelconque des revendications précédentes, comprenant en outre l'application d'un traitement thermique.

6. Procédé selon la revendication 5, comprenant en outre la soumission de l'arrêt de bille (27) à des températures élevées pendant le traitement thermique.

7. Procédé selon la revendication 5 ou 6, comprenant en outre la localisation du traitement thermique à une partie limitée du trépan à molettes coniques (11) qui comprend la soudure (29) et la région périphérique (23).

8. Procédé selon la revendication 5, comprenant en outre la soumission de la totalité du trépan à molettes coniques (11) au traitement thermique.

9. Procédé selon l'une quelconque des revendications 1 à 4, comprenant en outre l'application d'un traitement de vibration ultrasonique à la barrière (29) et à la région périphérique (23).

10. Procédé selon l'une quelconque des revendications précédentes, dans lequel ladite étape d'enlèvement de matière de la soudure comprend la formation d'un trou (39) dans la soudure (29) qui s'étend dans une direction axiale du chemin de bille (21).

11. Procédé selon l'une quelconque des revendications précédentes, dans lequel les contraintes résiduelles dans la soudure (29) et la région périphérique (23) sont réduites pour augmenter une capacité de charge d'exploitation et une durée de vie du trépan à molettes coniques.

12. Trépan à molettes coniques, comprenant:
un corps de trépan (13) pourvu de têtes (15) comportant des cônes (17), chaque tête et cône comprenant une piste de roulement (19) à une intersection entre la tête (15) et le cône (17), un chemin de bille (21) qui s'étend à partir de la piste de roulement (19) jusqu'à un diamètre extérieur de la tête (15), les pistes de roulement respectives de la tête et du cône étant alignées pour définir un espace toroïdal, des billes (25) situées dans la piste de roulement (19) pour retenir mécaniquement le cône (15) sur la tête (17), un arrêt de bille (27) situé dans le chemin de bille (21) pour retenir les billes (25) dans la piste de roulement (19), et une soudure (29) formée à proximité du diamètre extérieur de la tête (15) pour fixer l'arrêt de bille (27) dans le chemin de bille (21);
**caractérisé en ce que:**
ladite soudure comprend un vide (39).

13. Trépan à molettes coniques selon la revendication 12, dans lequel le vide (39) dans la soudure (29) est un trou qui s'étend dans une direction axiale du chemin de bille.

14. Trépan à molettes coniques selon la revendication 12 ou 13, comprenant en outre une soudure intérieure (31) formée à partir d'une première matière à proximité de l'arrêt de bille (27), la soudure (29) est formée sur la soudure intérieure (31) à partir d'une seconde matière dont la résistance est supérieure à celle de la première matière.

15. Trépan à molettes coniques selon la revendication 14, dans lequel la première matière est sélectionnée dans le groupe comprenant le nickel, un alliage de nickel, l'acier inoxydable et l'inconel; et la seconde matière est l'acier.
